

May 13, 1958

H. A. GREIS ET AL

2,834,077

METHOD OF PRODUCING PATTERNS FOR CORED CASTINGS

Filed May 28, 1954

FIG. 5.



FIG. 1.

FIG. 2.



FIG. 3.



FIG. 4.

FIG. 6.



20.

FIG. 7.



INVENTORS  
H. A. Greis  
BY J. R. Watson  
Sieber & Sieber  
ATTORNEYS.

1

2,834,077

**METHOD OF PRODUCING PATTERNS FOR CORED CASTINGS**

Howard A. Greis, Cedar Grove, N. J., and John R. Watson, Wauwatosa, Wis.

Application May 28, 1954, Serial No. 433,054

3 Claims. (Cl. 22—194)

The invention relates in general to improvements in the foundry art, and relates more specifically to an improved method of fabricating patterns and cores for the production of castings having internal passages or ducts.

The primary object of the present invention is to provide an improved method of economically producing durable castings having accurately formed and smooth internal conduits of diverse shapes, from various types of castable metals and other materials.

In various industries and especially in the manufacture of hydraulic, pneumatic and other fluid conducting manifolds and other cored castings, it is frequently necessary to provide castings each having one or more passages or spaces of diverse dimensions and shapes, some of which are interconnected while others are independent. Heretofore, such castings have been produced either by utilizing the usual patterns and cores to form the final casting molds, or by employing plastic patterns in so-called investment casting methods to provide the required cored spaces in the molds. With prior investment casting methods involving the use of molded plastic patterns, the patterns were of necessity made in configurations that could be readily withdrawn from the pattern mold. These patterns were used to form simultaneously both the internal and external casting surfaces, with the result that only short, simply shaped passages could be formed, except by tedious and costly mold fabrication techniques. However, all of these prior methods of fabricating such patterns and castings are expensive and slow while also resulting in the production of numerous defective molds and castings.

It is therefore an important object of this invention to provide an improved process of manufacturing cast hydraulic manifolds or the like, by facilitating the construction of the patterns for the fluid conducting passages and insuring the formation of smooth and unobstructed ducts in a rapid and inexpensive manner.

Another important object of the present invention is to provide a method of fabricating conduit cores of any desired length and configuration for molds utilized to produce castings embodying such cores, and wherein the formation of the cores is effected with the aid of patterns constructed from readily available materials.

A further important object of the invention is to provide an improved mode of producing castings having one or more smooth surfaced ducts therein, from diverse metals or castable material, by utilizing a plastic or other easily removable shell to form a refractory core for each of the required ducts and by eliminating these shells before the cores are applied to the final mold.

Still another important object of our present invention is to provide a simplified and inexpensive system for producing castings having a variety of internal passages of diverse lengths, cross sections and shapes, with accurately formed core patterns devoid of objectionable cavities or other defects.

An additional important object of this invention is to provide various improvements in the art of fabricating

2

extremely durable hydraulic manifold castings or the like, having smooth and unobstructed straight, curved or otherwise formed conduits emanating therefrom and crossing each other if desired, and which may be expediently manufactured to withstand high pressures.

These and other more specific objects and advantages of the present invention will be apparent from the following detailed description.

A clear conception of the several steps involved in the commercial exploitation of our invention and several modifications thereof, may be had by referring to the drawing accompanying and forming a part of this specification wherein like reference characters designate the same or similar parts in the various views.

Fig. 1 is a central longitudinal section through a typical composite core pattern or shell for producing an elongated conduit core having opposite end elbows and a medial off-set connected with the elbows by straight tubular portions;

Fig. 2 is a similar section through the pattern or shell of Fig. 1, but showing the same inverted and initially filled with a mass or core forming material;

Fig. 3 is another similar section through the core laden pattern or shell of Fig. 2, but with the shell provided with local stress relieving incisions or cuts;

Fig. 4 is an elevation of the molded core produced with the several steps depicted in Figs. 1, 2 and 3, but with the pattern shell removed;

Fig. 5 is a perspective view of a pattern or shell somewhat similar to that illustrated in Fig. 1, but which has been split along a longitudinal central plane in order to effect assembly thereof and removal from the cores for reuse;

Fig. 6 is a vertical central section taken through a typical completed mold showing several different types of conduit cores constructed in accordance with the invention, mounted therein preparatory to the production of a casting embodying passages simulating the cores; and

Fig. 7 is a transverse vertical section through the mold and core assemblage of Fig. 6 showing the cores in elevation.

While the invention has been shown and described herein as being especially advantageously applicable in the production of cast hydraulic manifolds having internally smooth passages or ducts communicating through elbows with one or more faces of each manifold, it is not the intent to unnecessarily restrict the improved production method to such field or industry; and it is also contemplated that specific descriptive terms employed herein be given the broadest possible interpretation consistent with the disclosure.

In accordance with this invention and as illustrated in the drawing, each individual conduit pattern or shell may consist of a single tube or it may be built up from one or more extruded or cast internally smooth tube sections 8, 9 of the desired internal cross section and cut to specific lengths and having elbows or fittings 10, 11 of any suitable configuration secured to the outer ends of the tube sections 8, 9 so as to provide smooth internal joints at the adjoining ends of the tubes and fittings as illustrated in Fig. 1. The inner or adjacent ends of the tube sections 8, 9 may be likewise interconnected by another fitting 12 of like internal cross section, to provide an off-set in the pattern, but the tubular shell may if desired, be produced from a single tubular section connected to the end fittings 10, 11 and the requisite off-sets may be produced by locally bending this single continuous section. In any event, the interior of each pattern must substantially conform with the external dimensions of the core which is to be produced, and should have

a smooth internal surface devoid of objectionable interruptions, cavities or projections.

When constructing these core patterns or shells it is preferable to utilize extruded plastic tubing and cast or extruded fittings formed of either plastic, wax, or any other suitable material, which is relatively solid and rigid under normal conditions, and can, preferably, be readily formed, molded or extruded, but which may be split into parts or disbursed either by heating or chemically, or otherwise. The shell forming material preferably should also be sufficiently transparent so that the internal surfaces thereof can be inspected and that the introduction of core forming material may be observed. It is also preferable to employ pattern forming substance which may be readily cut, and distorted when subjected to heat, and the several sections 8, 9 and fittings 10, 11, 12 may be united by cementing, welding or otherwise.

In order to produce a typical pattern or shell such as shown in Fig. 1, it is first necessary to determine the dimensions of the core which it is desired to form, after which plastic tubing of the proper internal cross section should be provided and either secured to the ends of a pre-formed fitting 12, or bent to provide the desired offset. The tubular sections 8, 9 should then be cut to proper length whereupon the end elbows 10, 11, if required, should be applied to the cut outer ends of the sections 8, 9. If the shell is to be expendable during removal from the core, the pattern will be complete upon attachment of the elbows; but in cases where it is desired to save the shell for re-use, it may be split longitudinally as in Fig. 5 into two or more parts 14, 15 adapted to be clamped together while the core forming material is being inserted, and to be subsequently separated in order to remove the molded core.

With the above described initial step of the present method, either destructible or re-usable patterns may be readily produced from plastics, waxes, or the like, with the aid of standard tubing and fittings of various internal cross-sections and lengths, and the interiors of these shells may be formed smooth and of substantially the shape of the desired cores. It is important to note that the interiors of these patterns or shells determine the final shapes of the cores while the exteriors thereof have no effect on these cores, and that a wide variety of patterns or shells may be produced without utilizing special and costly dies.

After each pattern has been thus produced, the next step is to fill the same with refractory core forming material 17. This material may be either a liquid slurry of refractory substance adapted to set by chemical action or hydration, or a semi-fluent relatively dry refractory substance likewise adapted to set or held sufficiently firm by bonding agents within the refractory, and in either case introduction of the material may be facilitated by inverting the shell as in Fig. 2. Any refractory core forming material which is of sufficient strength to retain its shape during pattern removal and core baking, may be utilized, and in either case the pattern must be completely filled with material 17 so that no voids or air pockets remain on the core surface. By utilizing transparent material in forming the shells, loading of the latter with refractory material 17 is also facilitated especially when producing cores of relatively small cross-section and of great length and having several medial bends therein. Examples of refractory materials 17 which may be used, are gypsum, other plaster compounds, or clay for producing aluminum or bronze castings, and substances such as ethyl silicates when producing other metal castings; and the proper positioning of the cores within the molds during casting is also important as will be later explained.

When split patterns or shells such as shown in Fig. 5 are utilized, the cores 17 when set may be readily removed by merely releasing the clamps from the parts 14,

15 and by separating these parts. However, in cases where the number of similar cores 17 required does not warrant the provision of split shells or patterns, these shells may be removed by burning, cutting, stripping, or 5 chemical action. In cases where the patterns are to be thus expended or destroyed when being removed from the cores 17, provision may be required to prevent possible distortion or destruction of the cores during removal, especially when removed by heating. The removal of the 10 patterns by heating or burning is also preferable since it combines drying of the cores 17 with the removal while the shells are being melted or burned off, but in order to permit the plastic patterns to shrink without detrimentally affecting the confined cores 17 it is preferable 15 to provide a series of local stress relief incisions or cuts 19 as illustrated in Fig. 3. The pattern and core assemblages may then be heated to elevated temperatures whereupon the plastic shells will be melted or burned off and the finished and relatively dry cores 17 shown in Fig. 20 4 will result.

Before the set cores 17 are finally applied to a mold 20 as in Figs. 6 and 7, they should be baked in an oven so as to insure complete dehydration and also to complete any chemical action which might take place in the 25 core forming material. The cores 17 may then be attached to a base section 21 of the mold 20, the sides and bottom of which determine the size and shape of the casting desired and which has an upper opening 22 which serves as a riser for the casting. The cores 17 should 30 also be positioned as shown, with the elongated medial portions thereof inclined relative to the fluid level of the molten metal, in order to facilitate the escape of gases and to avoid gas confining pockets, and when the cores have been properly positioned the entire mold assembly 35 should be heated before the final pouring operation takes place. The final casting may thereafter be effected with the pressure of the admitted casting material sufficiently high to force entrapped gases from the mold 20 and to obtain intimate contact of this metal with the smooth 40 surfaces of the cores 17, and the temperatures of the metal should also be properly controlled in accord with normal foundry procedure.

It has been found that by following the foregoing 45 steps, intricate castings of metal and other castable materials and having exceptionally smooth and accurately formed cored internal surfaces may be economically produced with minimum effort and great dependability. When re-usable split patterns comprising separable parts 50 14, 15 are utilized, these parts should be formed more durable and somewhat thicker than when expendable shells are employed, but the important feature of the improved method is the formation of smooth surfaced patterns and cores for producing internal smooth and accurately shaped cored surfaces on the final castings. 55 The patterns or shells are utilized only to produce the cores and not the castings, and need not be introduced within the molds, but it is also important when assembling cores within the molds to make proper provision for avoiding entrapment of gases. When employing patterns which are removed by heating, it is also important 60 to prevent distortion or destruction of the cores 17 due to shrinkage of the shells during pattern removal, and the improved method has proven highly satisfactory and successful in actual use. It is also noteworthy that the 65 present improved method makes it possible to produce molds with composite patterns some parts of which are formed of plastic while other parts are formed of different materials ordinarily utilized in pattern construction. This procedure enables the more intricate parts of 70 the patterns to be readily produced at low cost of the plastic material, while other more simple parts may be likewise produced by ordinary pattern making methods.

It should be understood that it is not desired to limit this invention to the exact steps of the method herein 75 shown and specifically described, for various modifica-

tions within the scope of the appended claims may occur to persons skilled in the art.

We claim:

1. The method of producing a mold for casting a unitary flat manifold having therein several segregated and crossing fluid conducting conduits terminating at a flat side of the final casting, which comprises, endwise uniting straight and arcuate end and medial sections of tubing formed of plastic having uniform wall thickness and smooth interiors to provide an independent pattern for each conduit having the same configuration and dimensions as those of the required final conduit, completely filling each tubular pattern with self-hardening refractory core forming material and after said material has hardened removing the plastic pattern from each hardened core having curved ends formed by said arcuate tube end sections, die molding a flat manifold cavity corresponding to the external shape of the final casting desired, and mounting the arcuate core ends at one side of the mold cavity to support the intermediate core portions within the cavity with arcuate medial portions thereof crossing but spaced from adjacent medial portions of other cores.

2. The method of producing a mold for casting a unitary flat manifold having therein several segregated and crossing fluid conducting conduits terminating at a flat side of the final casting, which comprises, endwise uniting straight plastic tubing sections with arcuate end and medial sections of similar tubing all having uniform wall thickness and smooth interiors to provide an independent pattern for each conduit having the same internal configuration and dimensions as those of the required final conduit, completely filling each tubular pattern with self-hardening refractory core forming material and after said material has hardened removing the plastic pattern from each hardened core having elbow ends formed by said arcuate tube end sections, molding a cavity corresponding to the external shape of the final casting desired and bounded on one side by a flat base board, and mounting the core elbow ends to position the

25  
30  
35  
40

intermediate core portions within the cavity with arcuate medial portions thereof crossing but spaced from adjacent medial portions of other cores.

3. The method of producing a mold for casting a unitary flat manifold having therein several segregated and crossing fluid conducting conduits terminating at a flat side of the final casting, which comprises, endwise uniting straight and arcuate end and medial sections of heat disbursable tubing having uniform wall thickness and smooth interiors to provide an independent pattern for each conduit having the same configuration and dimensions as those of the required final conduit, completely filling each tubular pattern with refractory core forming material and heating the assemblage to harden the confined material, thereafter removing the plastic pattern from each hardened core provided with elbow ends formed by said arcuate tube end sections, molding a cavity corresponding to the external shape of the final manifold desired, and mounting the core elbow ends at one side of the mold cavity to support the intermediate core portions entirely within the cavity with arcuate medial portions thereof crossing but spaced from adjacent medial portions of other cores.

References Cited in the file of this patent

UNITED STATES PATENTS

|           |              |                |
|-----------|--------------|----------------|
| 799,846   | Hay          | Sept. 19, 1905 |
| 1,034,334 | Bannister    | July 30, 1912  |
| 1,738,380 | Lukomski     | Dec. 3, 1929   |
| 1,761,522 | Elsey        | June 3, 1930   |
| 1,889,007 | Wallace      | Nov. 29, 1932  |
| 1,952,500 | Huetteman    | Mar. 27, 1934  |
| 2,136,404 | Wheeler      | Nov. 15, 1938  |
| 2,243,407 | Agnew        | May 27, 1941   |
| 2,456,424 | Neiman       | Dec. 14, 1948  |
| 2,510,417 | Rehklau      | June 6, 1950   |
| 2,531,496 | Bean         | Nov. 28, 1950  |
| 2,699,002 | Di Sylvestro | Jan. 11, 1955  |